

# UNITED STATES PATENT OFFICE.

ALFRED WEINGARTEN, OF BERLIN, GERMANY.

## METHOD OF PROCEDURE FOR SENSITIZING KINOFILMS FOR POSITIVE COPIES BY MEANS OF SOLUTIONS OF BICHROMATE.

No Drawing.

Application filed January 12, 1925. Serial No. 1,989.

*To all whom it may concern:*

Be it known that I, ALFRED WEINGARTEN, a citizen of Poland, residing at Berlin, Germany, have invented new and useful improvements in methods of procedure for sensitizing kinofilms for positive copies by means of solutions of bichromate, of which the following is a specification.

This invention relates to a method of procedure for sensitizing kinofilms for positive copies by means of solutions of bichromate. In comparison with the present state of technics this procedure has the advantage, that according to the new mode of procedure the duration of exposing to the light can be considerably reduced, and the durability of the sensitized film of gelatine is raised in comparison with the known methods of sensitizing by means of bichromates, as applicant has observed.

Essentially the procedure consists in sensitizing by means of a solution of bichromate the first celluloid layer coated with a layer of gelatine. According to the invention this layer is bathed in a solution of potassium bichromate, potassium ferro-

cyanide and potassium bromide (for instance—for 1 liter of solution 30 parts of potassium bichromate, 5 parts potassium ferro-cyanide and 5 parts potassium bromide). But the solution may be added to the colloid, before the latter is brought up to the celluloid band. Thereupon the sensitized layer is exposed to the light, washed by means of cold water and, then, developed in warm water, eventually upon previous colouring. With certain colloids the development can be obtained in a known manner without warm water; i. e. in a cold way. The not exposed gelatine swells, then, in such a measure, that the image becomes visible in the wet state.

What I claim is:—

A method of sensitizing kinofilms for positive copies, consisting in bathing the colloid in a solution of potassium bichromate, potassium ferro-cyanide and potassium bromide.

In testimony whereof I have signed my name to this specification.

ALFRED WEINGARTEN.